

June 8, 1954

A. E. VAN DORMAEL ET AL

2,680,686

SENSITIZED AND SUPERSENSITIZED PHOTOGRAPHIC EMULSIONS

Filed Jan. 31, 1950

2 Sheets-Sheet 1

A = A COMPOUND OF FORMULA V.

B = A DYE OF FORMULA XI.

Fig. 1. C = THE COMPOUND OF FORMULA V  
WITH THE DYE OF FORMULA XI.



D = A COMPOUND OF FORMULA VIII.

E = A DYE OF FORMULA XII.

Fig. 2. F = THE COMPOUND OF FORMULA VIII  
WITH THE DYE OF FORMULA XII.



G = A COMPOUND OF FORMULA V.

H = A DYE OF FORMULA XIII.

Fig. 3. I = THE COMPOUND OF FORMULA V  
WITH THE DYE OF FORMULA XIII.



June 8, 1954

A. E. VAN DORMAEL ET AL

2,680,686

SENSITIZED AND SUPERSENSITIZED PHOTOGRAPHIC EMULSIONS

Filed Jan. 31, 1950

2 Sheets-Sheet 2

J = A COMPOUND OF FORMULA V.

K = A DYE OF FORMULA XIV.

Fig. 4. L = THE COMPOUND OF FORMULA V  
WITH THE DYE OF FORMULA XIV.



M = A COMPOUND OF FORMULA IX.

N = A DYE OF FORMULA XXIV.

Fig. 5. O = THE COMPOUND OF FORMULA IX  
WITH THE DYE OF FORMULA XXIV.



Inventors  
André Emile Van Dormael  
Jean Marie Stys  
By Richard L. L.

Aug 7

## UNITED STATES PATENT OFFICE

2,680,686

SENSITIZED AND SUPERSENSITIZED  
PHOTOGRAPHIC EMULSIONS

André Emile Van Dermael, Heverlee-Louvain,  
Jean Marie Nys, Louvain, and Arthur Henri  
De Cat, Kessel-Loo-Louvain, Belgium, assignors  
to Gevaert Photo-Producten, N. V., Mortsel,  
Belgium, a Belgian company

Application January 31, 1950, Serial No. 141,601

Claims priority, application France  
February 1, 1949

2 Claims. (Cl. 95—7)

1

The present invention relates to a process for the production of photographic silver halide emulsions.

This invention more particularly relates to the sensitization and supersensitization of photographic silver halide emulsions.

An object of the present invention is to provide a new process for sensitizing and supersensitizing photographic emulsions.

A further object is to provide a photographic element comprising an emulsion sensitized or supersensitized according to our new process.

Other objects will appear from the following description.

We have found that the sensitivity of photographic silver halide emulsions optionally containing optical sensitizers may be improved by incorporating into these emulsions products corresponding to the following general formula



wherein

D=the atoms necessary to complete a member selected from the group consisting of five- and six-membered heterocyclic nuclei and five- and six-membered heterocyclic nuclei bearing a fused-on arylene ring,  
n=a positive integer of from 1 to 2.



The following examples serve to illustrate the invention without limiting, however, the scope thereof.

*Example 1*

A silver bromo-iodide emulsion, containing per kg. of emulsion 10 mg. trimethincyanine of the formula



is strongly supersensitized by simultaneously using 30 mg./kg. of the compound of the formula



R=a member selected from the group consisting of H, alkyl, substituted alkyl, aryl, alkenyl and alkylene,

R'=a member selected from the group consisting of a substituted acyl group, a not substituted acyl-group, a substituted amido group and a not-substituted amido group.

The compound of said general formula wherein R=H may also correspond to the tautomeric formula



The compounds corresponding to the first given general formula wherein R'=an acyl group, substituted or not, may be obtained for instance by condensation of a base bearing an imino group and corresponding to the formula



45 which may be synthesized in the following manner: A mixture of 2 g. N-methyl-2-imino-dihydrobenzthiazole and 0.8 g. ethyl-malonate is heated at 170° C. for 1 hour. After cooling, the product obtained is sucked off and dried. Melting point (after recrystallisation from alcohol): 262-263° C.

*Example 2*

55 The spectral sensitivity of a silver chloride

3

emulsion is increased by using 50 mg./kg. of the compound of the formula



prepared as follows: 5 g. N-phenyl-2-imino-dihydrobenzthiazole in 50 cm.<sup>3</sup> acetic anhydride are heated at boiling temperature. After cooling, the product is precipitated by water. Melting point (after recrystallisation from alcohol): 149.5-150.5° C.

*Example 3*

A silver bromo-iodide emulsion, containing per kg. of emulsion 25 mg. trimethincyanine of the formula



is supersensitized by simultaneously using 30 mg./kg. of the compound of the formula in Example 2.

*Example 4*

A silver bromide emulsion, containing per kg. of emulsion 20 mg. cyanine of the formula



is supersensitized by simultaneously using 30 mg./kg. of the derivative of the formula



which may be prepared as follows: A suspension of 5 g. N-methyl-2-imino-dihydrobenzthiazole in 40 cm.<sup>3</sup> acetic anhydride is refluxed for 15 minutes. After adding 100 cm.<sup>3</sup> diluted alcohol (70%) the mixture is heated once more at boiling temperature for 5 minutes whereafter the product is precipitated by ice-water. Melting point (after recrystallisation from alcohol): 141-142° C.

*Example 5*

A silver chloride emulsion, containing per kg. of emulsion 6 mg. trimethincyanine of the formula



is strongly supersensitized by simultaneously using 30 mg./kg. of the derivative of the formula



which may be prepared as follows: A mixture of 1.6 g. N-methyl-2-imino-dihydrobenzthiazole and 2.2 g. 2-benzthiazolyl ethyl acetate in 2 cm.<sup>3</sup> xylene is refluxed for 4 hours in the presence of 1 drop of piperidine. After cooling, the precipitate thus formed is sucked off and recrystallized from alcohol. Melting point: 172-173° C.

*Example 6*

A silver bromide emulsion, containing per kg. of emulsion 25 mg. trimethincyanine of the formula



is supersensitized by simultaneously using 30 mg./kg. of the compound of the formula



prepared in the following manner: A mixture of 3.2 g. N-methyl-2-imino-dihydrobenzthiazole and 4.2 g. benzoyl chloride in 35 cm.<sup>3</sup> xylene is refluxed for 3 hours. After cooling, the precipitate formed is recrystallised from diluted alcohol. Melting point: 156.5-157.5° C.

*Example 7*

A silver chloride emulsion, containing per kg. of emulsion 20 mg. trimethincyanine of the formula



is supersensitized by simultaneously using 30 mg./kg. of the compound of the formula



obtained as follows: A mixture of 3 g. N-methyl-2-imino-dihydrobenzthiazole and 10 cm.<sup>3</sup> ethyl aceto acetate is refluxed for 2 hours. After cooling, the crystals formed are sucked off. Melting



## Example 13

A silver bromo-iodide emulsion, containing per kg. of emulsion 20 mg. trimethincyanine of the formula



is supersensitized by simultaneously using 30 mg./kg. of the compound of the formula



prepared as follows: A mixture of 1.4 g. 2-amino-benzoxazole (according to Skraup, Ann. 419 (1919) 68) and 1.4 g. benzoylchloride in 25 cm.<sup>3</sup> dry benzene, is refluxed for 30 minutes. Then 0.8 g. pyridine are added to the reaction mixture which is further refluxed for 3 hours. After filtering while still warm, the filtrate is cooled and the precipitate formed is filtrated. Melting point (after recrystallisation from alcohol) 214–215° C.

## Example 14

A silver chloro-bromide emulsion, containing per kg. of emulsion 10 mg. trimethincyanine of the formula



is supersensitized by simultaneously using 30 mg./kg. of the compound of formula



prepared according to Camps, Archiv der Pharmazie, 240 (1902) 363.

## Example 15

A silver chloro-bromide emulsion, containing per kg. of emulsion 10 mg. trimethincyanine of the formula



is supersensitized by simultaneously using 30 mg./kg. of the compound of the formula



prepared as follows: A mixture of 4 g. N-methyl-2-imino-dihydrobenzothiazole and 37.5 cm.<sup>3</sup> hydroquinone-diacetylchloride in 45 cm.<sup>3</sup> xylene is refluxed for 3 hours. After cooling, the crystalline product is separated and recrystallised from cyclohexanone. Melting point: 276–277° C.

## Example 16

10 A silver chloride emulsion, containing per kg. of emulsion 15 mg. cyanine according to the formula



15 is supersensitized by simultaneously using 30 mg./kg. of the compound of the formula



20 prepared as follows: A mixture of 0.8 g. N-methyl-2-imino-dihydrobenzothiazole and 1.1 g. 2-carbethoxymethyl-benzothiazole in 1 cm.<sup>3</sup> xylene, is heated for 4 hours at boiling temperature in the presence of 5 drops pyridine. After 25 cooling and recrystallising from butanol, a prod-

35 product is obtained, melting at 172–173° C., and corresponding to the formula



40 50 2 g. of this compound and 1.12 g. methyl iodide are heated at 100° C. for 48 hours in a sealed tube and a product of the formula



55 is obtained. Melting point: 253–254° C. (with de-

composition). 1 g. of the latter product is dissolved in 50 cm.<sup>3</sup> phenol and 50 cm.<sup>3</sup> anhydrous



9

alcohol. After adding 2 g. KOH dissolved in 20 cm.<sup>3</sup> ethanol, the reaction mixture is refluxed for 2 hours. On pouring out into sodium hydroxide N, the azaketomethylene compound corresponding to the formula



precipitates. Melting point (after recrystallisation from isoamyl alcohol): 326–327° C.

The specification is accompanied by drawings to illustrate the supersensitizing effect obtained with five of our new dyestuff combinations used in silver halide emulsions. Each of the Figs. 1 to 5 is a diagrammatic reproduction of three spectrograms. In each figure, the sensitivity is represented by a dotted line; the sensitivity of the emulsion containing only the cyanine dye is represented by a dash-dotted line; and the sensitivity of the emulsion containing the compound according to the invention in combination with the cyanine dye is represented by the solid line. 25

We claim:

1. A photographic silver halide emulsion containing the compound of the formula



10

2. A photographic silver halide emulsion containing the combination of the dyestuff of the formula



10 and the dyestuff of the formula



References Cited in the file of this patent

UNITED STATES PATENTS

| Number    | Name           | Date          |
|-----------|----------------|---------------|
| 2,080,049 | Kendall        | May 11, 1937  |
| 2,153,930 | Kendall        | Apr. 11, 1939 |
| 2,177,635 | Carroll et al. | Oct. 31, 1939 |
| 2,298,732 | Brooker et al. | Oct. 13, 1942 |
| 2,312,040 | Kendall et al. | Feb. 23, 1943 |
| 2,340,882 | Kendall        | Feb. 8, 1944  |
| 2,490,745 | Carroll et al. | Dec. 6, 1949  |
| 2,503,861 | Weissberger    | Apr. 11, 1950 |

## FOREIGN PATENTS

Number                   Country                   Date  
617,720           Great Britain       Feb. 10, 1949